# EUROPEAN PATENT SPECIFICATION

(11) **EP 2 662 167 B1**
(45) Date of publication and mention of the grant of the patent: **22.03.2017**
(21) Application number: 13179763.1
(22) Date of filing: 21.11.2008
(51) Int. Cl.: B22F 3/15, C22C 1/04

(54) **Hot pressed net or near net shape powder component**
Heiß gepresstes, Endkontur- oder endkonturnahes Pulverbauteil
Composant de poudre à forme définitive ou presque définitive, compressé à chaud

(30) Priority: 22.11.2007 GB 0722850; 23.01.2008 US 22935 P
(43) Date of publication of application: 13.11.2013
(62) Divisional of application: 08852655.3
(73) Proprietor: Advanced Interactive Materials Science Limited, Edgbaston Birmingham B15 3BH (GB)
(72) Inventor: ARCHER, Geoffrey Frederick, Stamford, Lincolnshire PE9 4BA (GB)
(74) Representative: Stratagem IPM Limited

(56) References cited:
- GB-A- 846 292
- GB-A- 941 795
- US-A1- 2004 055 416

## Description

### Field of the Invention

This invention relates to a net or near net shape powder metallurgy process.

The invention relates particularly, but not exclusively, to the provision of an atomic diffusion filter between a graphite former, used to derive the finished net or near net shape form used in the manufacture of near net shape powder metallurgy components.

### Background to the Invention

A known manufacturing method used for producing components and materials utilises the consolidation of metal powders by Hot Isostatic Pressing. A pre-consolidation of the metal powders may or may not be used utilising Cold Isostatic Pressing.

In summary, metal powder is placed in a containment and a vacuum is applied within the containment, and the containment is sealed. This then may or may not be partially consolidated in a cold form by subjecting the containment to a cold Isostatic process (CIPing). The contained powder is then subjected to Hot Isostatic Pressing (HIPing).

The HIPing process utilises the application of heat at approximately, but not essentially, 80% of solidus of the material of which the powder is derived. This process subjects the metal powder to thermo mechanical stress whereby the metal powders are mechanically deformed in a super plastic condition. The resulting intimate contact and movement between the powder particles results in a shear and compressive stresses being placed upon them. As result of this process an atomic interaction (interdiffusion) between the particles takes place subsequently removing all prior practical history thus creating a solid homogenous metal form.

There is a need with certain components to be able to create an accurate and/or near accurate final shape to the component being manufactured. This can be done using a graphite former machined to an accurate size.

We have appreciated that it is desirable to partially inhibit or limit (filter) the diffusion of carbon atoms from the graphite into the powdered metal being processed.

US2004/055416 describes hot isostatic pressing of a homogenously mixed composition of copper and carbon.

GB941795 describes a sintered metal powder compressed by way of a rolling process.

### Statements of Invention

According to the invention there is provided the net or near net shape component of claim 1.

Preferably the nickel based alloy has the following composition by weight percent: C 1.0, Cr 15, Si 4.0, B 3.5, Fe 4.5, Ni balance.

Preferably the component is greater than 2 metres in length.

Preferably the component is a motor or pump.

### Examples in accordance with the invention

(A) In the case of graphite forms used to produce net/near-net-shapes in PM Nickel based alloys containing for example Cr, Fe, B, Si, C 5 thin aqueous layers of BN of between 1µm and 2 µm per layer work satisfactorily. This allows a controlled amount of carbon to diffuse into the Ni alloy to depth of between 100µm and 500µm. This slightly increases the size of the precipitated CrC within this 100µm band and thereby increasing the macro hardness from nominally 55R_{c} to approximately 57R_{c}. This slight increase in hardness increases the abrasive wear resistance of the consolidated material whilst limiting brittle behaviour. Coatings built of multi layers from 1µm to up to and beyond 250µm have been applied to control and tailor the surface morphology and properties of consolidated materials.
   Also in this particular application of the invention the BN layer also acts as a release agent allowing the graphite former to be removed following HIPing. Here the surface finish of the net shape part is important. Therefore it is of additional importance to ensure that the BN layer is deposited evenly and accurately.
**(B)** Thin shell net shape profiled bore walls can be produced for the high performance automotive industry. These parts are required to be manufactured in high quality ferrous steel alloy, and in this particular application of the invention it is essential to control the level of carbon diffusion into the surrounding steel part and to keep it as low as possible. Whilst in this case the accuracy is not so important, the quality and subsequent performance of the material is of great importance. The BN diffusion barrier in this application is applied to a thickness that is so chosen as to reduce carbon diffusion into the steel to an insignificant level.
**(C) Choice of Suitable Alloys for Surface Treatment**
   Typical materials suitable for surface modification by the diffusion of carbon are nickel-based alloys containing Si, B, Fe, Cr and C in this case the carbon content of the alloy is enhanced by the diffusion of further carbon during the HIPing process. It may be desirable to adjust the specified carbon and/or chromium content to optimise the post process properties of the material.

It has been found beneficial to orchestrate the diffusion of carbon into a number of nickel and ferrous-based materials but Alloy steels designed specifically for carburising are in particular suitable for use in this application.

A Nickel based alloy is typically:-
C1.0, Cr15, Si 4.0, B3.5, Fe4.5 Ni Balance, by weight percent.

A Ferrous alloy is typically;
C 0.13, Si 0.20, Mn 0.50, P 0.020, S 0.020. Mo 0.18, Ni 3.40, by weight percent.

In addition specific material composition can be compiled to optimise the process potential for a particular requirement

The diffusion of carbon into other alloy steels followed by an appropriate heat treatment may be beneficial to increase both stiffness and the surface performance of components even though the materials are not ordinarily treated in such a way.

In all cases the duration of the peak HIPing temperature can be adjusted to optimise the depth of carbon diffusion; provided the increase in time does not have a detrimental effect upon the overall morphology of the consolidated material. For example increased grain growth and/or undesirably affect the volume fraction or dimensions of precipitates.

## Claims

1. A net or near net shape component, produced by a hot isostatic pressing process or hot uniaxial pressing process, the component having a solid homogenous metal form and a modified surface in which the surface of the component incorporates a controlled amount of carbon that has diffused into the surface from a graphite former during pressing, **characterized in that** the component is made from a nickel alloy.

2. The component of claim 1 in which the Nickel based alloy has the following composition by weight percent: C 1.0, Cr 15, Si 4.0, B 3.5, Fe 4.5, Ni balance.

3. The component according to claim 1 or claim 2 which is greater than 2 metres in length.

4. The component according to claims 1-3 which is a linear motor or pump.

## Patentansprüche

1. Eine Endkontur- oder endkonturnahe Komponente, die mittels eines heißisostatischen Pressvorgangs oder eines uniaxialen Heißpressvorgangs hergestellt wird, die Komponente hat dabei eine feste homogene Metallform und eine modifizierte Oberfläche, die Oberfläche der Komponente enthält eine kontrollierte Menge von Kohlenstoff, der beim Pressen aus einem Graphitformer auf die Oberfläche diffundiert, **dadurch gekennzeichnet, dass** die Komponente aus einer Nickellegierung besteht.

2. Die Komponente gemäß Anspruch 1, in der die Legierung auf Nickel-Basis die folgende Zusammensetzung nach Massegehalt hat: C 1,0, Cr 15, Si 4,0, B 3,5, Fe 4,5, Ni Gleichgewicht.

3. Die Komponente gemäß Anspruch 1 oder Anspruch 2, die größer als 2 Meter in der Länge ist.

4. Die Komponente gemäß Anspruch 1-3, die ein Linear-Fahrmotor oder eine Pumpe ist.

## Revendications

1. Un élément de forme nette ou presque nette, produit par un procédé de compression isostatique à chaud ou un procédé de compression uniaxiale à chaud, l'élément présentant une forme de métal homogène solide et une surface modifiée dans laquelle la surface de l'élément incorpore une quantité contrôlée de carbone qui a diffusé dans la surface à partir d'un gabarit en graphite pendant la compression, **caractérisé en ce que** l'élément est fabriqué à partir d'un alliage de nickel.

2. L'élément selon la revendication 1, dans lequel l'alliage à base de nickel présente la composition suivante en pourcentage de poids : C 1,0, Cr 15, Si 4,0, B 3,5, Fe 4,5, Ni en complément.

3. L'élément selon la revendication 1 ou la revendication 2 qui est supérieur à 2 mètres de longueur.

4. L'élément selon les revendications 1 à 3 qui est un moteur linéaire ou une pompe.
